

March 25, 1958

W. SONNENSCHEIN

2,828,229

CELLULOSE FIBRES COATED WITH COTTON WAX

Filed Dec. 14, 1954

2 Sheets-Sheet 1



INVENTOR.  
WILHELM SONNENSCHEIN

BY

*Andreas S. Haas*

ATTORNEY

March 25, 1958

W. SONNENSCHEIN

2,828,229

CELLULOSE FIBRES COATED WITH COTTON WAX

Filed Dec. 14, 1954

2 Sheets-Sheet 2



INVENTOR.  
WILHELM SONNENSCHEIN  
BY  
*Frederick L. Haag*  
ATTORNEY

1

2,828,229

## CELLULOSE FIBRES COATED WITH COTTON WAX

Wilhelm Sonnenschein, Kassel, Germany, assignor to  
Spinnfaser Aktiengesellschaft, Kassel-Bettenhausen,  
Germany, a corporation of Germany

Application December 14, 1954, Serial No. 475,247

Claims priority, application Germany December 18, 1953

1 Claim. (Cl. 117—139.5)

This invention relates to the manufacture of regenerated cellulose staple fibers; and in particular is directed to a novel process for the finishing of said fibers.

It is a well-known fact that the properties and manipulability of fibers and threads are greatly affected by the finish thereon. Manufacturers of rayon staple apply compositions thereto in order to impart a soft hand and to improve its spinning qualities. Such application is generally designated as "finish"; and accordingly, the term "finish" and "finishing" as used herein means the treatment applied in the manufacture of rayon staple. The term "lubrication" is used in the textile industry, as contrasted with "finish" as above defined, to designate the additional lubrication applied in the textile mill. The purpose of the finishing, therefore, is to provide a staple that will card, comb, and particularly draw and spin better than unfinished staple.

It is also known that the preparation of the stock for spinning on the worsted system differs from that carried out on the woolen system. In the worsted system, the rayon is separately subjected to carding and combing from the raw stock stage until the rayon top is produced. That rayon top is then blended with the separately prepared woolen top in the subsequent drawing operation. In the woolen system, the rayon staple and the wool staple are generally blended in the early stages of the manipulation.

Blended cotton and rayon yarns are generally made by blending the different fibers. Blending in some cases takes place in the drawing stage that produces the roving; and in some cases the blending is initiated with the raw stock forms. When working with rayon staple alone on the cotton system, the lap, card sliver, comb sliver, roving and the ultimately spun yarn constitute 100 percent rayon.

The problem of "finishing" is of particular significance in connection with the working purely of rayon staple (cellulose wool). Whereas the spinning of cellulose wool on the worsted system and on the woolen system does not generally present any substantial difficulties due to the mixture of the synthetic fibers with the natural fibers so that the known finishing agents are adequate, the spinning of the rayon staple on the cotton system gives rise to difficult problems. The quality of the cotton type of spinning the rayon staple (cellulose wool) depends—in addition to other factors—very much upon the adhesiveness of the staple in the fleece and in the carding ribbon or sliver; and it is also dependent upon the attitude of these synthetic fibers when drawn into ribbons or slivers or rovings. The finishing agents which have been used heretofore have not been found successful for this purpose. For example, the card sliver made from staple finished with the usual finishing agents exhibits a jerky draw as shown in the graph of Fig. 1. The result thereof was that during the subsequent operations, periodic non-uniformities were to be expected in the yarn goods or the fabric.

In contrast thereto, a completely jerkless drawing is desired as indicated in the graph of Fig. 2; a smoothness of drawing that is characteristic for natural fibers possessing the well-known super molecular structure. Some of

2

the known cation active finishing agents do produce a jerkless drawing, but these agents so substantially reduce the adhesiveness of the fiber to the base that they are not suitable as finishing agents for cellulose wool.

5 It has been found that cellulose staple can be finished by means of suitable finishing agents so as to impart thereto the desired jerkless drawing characteristics. Investigations have shown that the higher aliphatic saturated alcohols having a carbon content of  $C_{22}$  to  $C_{34}$ , preferably  $C_{29}$  to  $C_{31}$  impart to the rayon staple the quality of jerkless drawing without appreciably reducing adhesiveness of the fibers within the ribbon or sliver. These alcohols may be, in part, esterified with higher fatty acids having a carbon content of from 15 to 34 carbon atoms. Furthermore, 15 mixtures of the aforementioned alcohols and esters of different chain alcohols may be used.

As starting materials for the manufacture of these alcohols and esters, either pure or in admixture with each other, various natural waxes may be used. For example, upon 20 partially saponifying beeswax, there is obtained a mixture of alcohols and esters, which mixture when used in an aqueous emulsion as a finishing agent imparts to synthetic fibers jerkless drawing. Among the natural waxes which are suitable in accordance with this invention, there are the cotton waxes in the form in which they are extracted from cotton. They are suitable for this purpose since they excel in their comparatively high content of free aliphatic alcohols. The admixture of about 20 percent of free high molecular fatty acids and paraffins to the aforementioned 25 alcohols and esters is not harmful. The alcohols or the ester-alcohol mixtures are emulsified in water by means of an emulsifying agent. The quantity of the emulsifying agent used for such purpose should be kept as low as possible. The amount of emulsifying agent should not exceed 30 5 percent as otherwise the presence of the emulsifying agent reduces the improved drawing effect produced by the finishing.

Alcohols such as myricyl alcohol ( $C_{31}H_{63}OH$ ) or behenic alcohol ( $C_{22}H_{45}OH$ ) are used in concentrations of 40 from 2.0 to 3.0 grams per liter of the finishing bath. The cotton waxes may be used in the same concentration.

Other natural waxes which do not contain an adequate content of the high molecular weight aliphatic alcohols, as for example, carnauba wax or beeswax, and the like, should 45 be subjected to a partial saponification. After acidification of the saponification mixture and separation of the organic constituents, the isolated saponification products may be used in the same concentrations as described above. Natural waxes of the type just mentioned which have a 50 content of free alcohols of less than 40 percent are not suitable for obtaining a jerkless draw since concentrations of 10 grams per litre and above must be used which result in sticking or adhesion of the individual fibers to each other 55 whereby the manufacture of a perfect thread or yarn is prevented.

Waxes, per se, have been used in the textile industry for different purposes. For example, by treatment of the 60 fibers with solutions of paraffin wax, beeswax or carnauba wax in solvents such as kerosene, the aim has been to impart better coherence to threads when wound up in the form of balls or rolls. It has also been proposed to impregnate threads by means of emulsions consisting of montan wax, oil and resin. In another method, textile 65 threads are generally treated with an emulsion containing paraffin, a hydrophilic agent and a hydrophobic agent to improve the slipping or gliding of the fibers. The paraffin in such cases may also be replaced by wax. It has been found that treatment with paraffin does not result in a cellulose wool card ribbon or sliver which can be drawn without jerkiness.

The success of the process in accordance with the instant invention will be further made apparent by the following examples and counter-examples.

*Example 1*

1.2 kg. of myricyl alcohol are molten together with 0.04 kg. of a wax-emulsifying emulsifier, as for instance, an emulsifier manufactured by the firm of Dr. Th. Böhme under the name "Special Emulsifier 1836." Then the mixture is left to cool while being continuously agitated.  $\frac{1}{2}$  liter of hot water is added in small quantities, the mixture being stirred to form a paste which is subsequently fed into about 400 liters of hot water having a temperature of 40° to 50° C. The mixture is then emulsified by means of an emulsifying device. The concentration of this bath is 3.0 grams per liter. It is charged with 20 kg. of rayon staple (cellulose wool); and treated for about five minutes. Then the moist fibers are squeezed to achieve a moisture content of about 140 percent; and the fibers are dried at 70° C. A card ribbon made from such synthetic fiber shows a drawing illustrated by the graph of Fig. 3.

*Example 2*

1.2 kg. of behenic alcohol are molten and 0.06 kg. of 96 percent sulphuric acid added thereto. The acid is allowed to act on the alcohol for about ten minutes while being stirred; and the mixture is cooled to room temperature. Then 5 liters of water are added to the mixture; and the mass neutralized with caustic soda; heated to 70° C.; and dispersed in 200 liters of water of 40° to 50° C. Cellulose wool treated therewith in accordance with the method of Example 1 develops a card ribbon drawing illustrated by the graph of Fig. 4.

*Example 3*

0.6 kg. of myricyl alcohol ester of cerotic acid ( $\text{CH}_3(\text{CH}_2)_{24}\text{COOH}$ ), 0.3 kg. of a saturated hydrocarbon fraction having a chain length of more than  $\text{C}_{30}$  and 0.05 kg. of a wax-emulsifying emulsifier, such as the Special Emulsifier 1836 of the firm of Dr. Th. Böhme, are molten together and allowed to cool while being continuously stirred. Then  $\frac{1}{2}$  liter of hot water is added in small quantities and the mass stirred to form a paste. This paste is introduced into about 200 liters of hot water having a temperature of about 40° to 50° C.; and emulsified by means of an emulsifying device. 10 kg. of synthetic fibers are fed into the bath.

*Example 4*

1.2 kg. of cotton wax are molten together with 40 grams of a wax-emulsifying emulsifier. The mixture is allowed to cool while being continuously stirred. By the continuous gradual addition of  $\frac{1}{2}$  liter of hot water, the mixture is stirred to form a paste. This paste is added to about 400 liters of hot water having a temperature of 40° to 50° C.; and emulsified by means of an emulsifying device. The concentration of this bath is 3 grams per liter. 20 kg. of cellulose wool are treated with this emulsion, the moisture content thereof is then reduced, by squeezing, to about 140 percent; and the fibers are dried at 70° C. A carded roving made from this cellulose wool shows a drawing illustrated by the graph of Fig. 5.

*Example 5*

2 kg. of an oxyethylated stearic acid oxyethylamide are introduced into 40 liters of water having a temperature of 70° C. The mixture is stirred for about  $\frac{1}{4}$  hour until emulsification is completed, and the emulsion is diluted with 1000 liters of water having a temperature of 50° to 60° C. 50 kg. of cellulose wool are placed in the emulsion; and the finishing agent allowed to act for about five minutes upon the fibers. After removal from the bath, the water is thrown off fibers until the moisture content thereof is reduced to about 130 to 140 percent. The fibers are dried in a drying oven having a temperature between 70° to 80° C. A carded roving made from these fibers shows a drawing illustrated by the graph of Fig. 1.

It will be understood that the foregoing description of the invention and the examples set forth are merely illustrative of the principles thereof. Accordingly, the appended claim is to be construed as defining the invention within the full spirit and scope thereof.

I claim:

As a new article of manufacture, rayon staple having thereon a "finish" of cotton wax.

**References Cited in the file of this patent**

| UNITED STATES PATENTS |           |                                 |
|-----------------------|-----------|---------------------------------|
| 40                    | 2,132,348 | Bertsch ----- Oct. 4, 1938      |
|                       | 2,141,845 | Schrauth ----- Dec. 27, 1938    |
| 45                    | 2,406,407 | Schiessler ----- Aug. 26, 1946  |
|                       | 2,596,985 | Cook et al. ----- May 20, 1952  |
| 50                    | 2,690,427 | Schalatter ----- Sept. 28, 1954 |

**OTHER REFERENCES**

Leaper et al.: "Textile Colorist," July 1932, 117-139.5 (pp. 441-445).